

## UNITED STATES PATENT OFFICE

2,128,782

PROCESS OF MANUFACTURING NON-IN-  
FLAMMABLE ARTICLES OF ORGANIC FI-  
BROUS MATERIALS

Bernhard Müller, Berlin-Charlottenburg, Germany, assignor to Rutgerswerke-Aktiengesellschaft, Berlin, Germany

No Drawing. Application October 26, 1936, Serial No. 107,646. In Germany December 14, 1935

7 Claims. (Cl. 92—21)

My present invention relates to a process of making non-inflammable plates, slabs, or other articles from fibrous materials, for instance from fibers of wood, straw or the like. According to my invention the fibrous materials from which plates, slabs or other articles are produced in a known manner, are soaked in an aqueous solution containing as essential components ammonia, water-soluble phosphates such as ammonium phosphate and water-soluble silicofluorides, especially magnesium silicofluoride. From such solutions difficultly soluble phosphates and silicic acid are precipitated on the fibers which are worked up to plates, slabs or the like in the usual way.

Example.—170 kilos of a mass consisting of a mixture of wood pulp and straw pulp are beaten in a hollander of a capacity of about 4 cbm. To the aqueous pulp 85 kilos of aqueous ammonia of 25% and 24 kilos of monoammonium phosphate ( $(\text{NH}_4\text{H}_2\text{PO}_4)$ ) dissolved in 110 kilos of water are added and uniformly distributed. Finally 57 kilos of magnesium silicofluoride ( $\text{MgSiF}_6 \cdot 6\text{H}_2\text{O}$ ) dissolved in 150 kilos of water are added in small portions, each portion being uniformly distributed in the aqueous mass. The pulp is beaten in the hollander for about 30 minutes and is then worked up in the usual manner to plates, slabs or the like.

The ammonium phosphate reacts in the presence of ammonia with magnesium silicofluoride according to the following equation:



The magnesium ammonium phosphate and the silicic acid are deposited in the fibers and render the plates, slabs or other articles, prepared from the fibrous mass, non-inflammable.

Instead of magnesium silicofluoride other salts of fluosilicic acid may be used such as zinc or aluminium silicofluoride and instead of monoammonium phosphate other ammonium phosphates or other water soluble salts of phosphoric acid such as sodium or potassium phosphates.

The plates, slabs or the like prepared according to my present invention show a marked resistivity against heat and fire. They char under the in-

fluence of strong heat, but they are non-inflammable and do not burn with a flame. This high resistivity against heat can only be attained if in accordance with my invention the fibers contain silicic acid beside a water insoluble metal ammonium phosphate.

What I claim is:

1. In a process of manufacturing non-inflammable articles of organic fibrous materials the steps of preparing an aqueous pulp of an organic fibrous material, adding to said pulp a solution containing as essential components ammonium hydroxide and a water soluble salt of phosphoric acid, selected from the group consisting of the phosphates of ammonium, sodium or potassium, admixing to the mixture thus obtained an aqueous solution of a water soluble metal salt of fluosilicic acid selected from the group consisting of the fluosilicates of magnesium, zinc and aluminum to precipitate a water insoluble metal ammonium phosphate and silicic acid on the fibres of said fibrous material, and then forming the treated pulp into non-inflammable articles.

2. A process according to claim 1, in which monoammonium phosphate is used as the water soluble salt of phosphoric acid and magnesium silicofluoride is used as the water soluble metal salt of fluosilicic acid.

3. A process according to claim 1, in which 1 mol. of monoammonium phosphate, 1 mol. of magnesium silicofluoride and 6 mols of ammonium hydroxide are used.

4. A process according to claim 1, in which monoammonium phosphate is used as the water soluble salt of phosphoric acid and zinc silicofluoride is used as the water soluble metal salt of fluosilicic acid.

5. A process according to claim 1, in which sodium phosphate is used as the water soluble salt of phosphoric acid.

6. A process according to claim 1, in which potassium phosphate is used as the water soluble salt of phosphoric acid.

7. A process according to claim 1, in which aluminum silicofluoride is used as the water soluble salt of fluosilicic acid.

BERNHARD MÜLLER.